

Nov. 12, 1935.

H. PELS

2,020,853

PHOTOGRAPHIC AMUSEMENT DEVICE AND METHOD OF MAKING THE SAME

Filed Sept. 27, 1933

Fig. 1



13

Fig. 2



16

Fig. 3



13

Fig. 4



10 After exposure and development

Fig. 5



10 After bleaching

Fig. 6



10 After restoration

INVENTOR

Herbert Pels,

BY

Fredrich Freitnfeld  
ATTORNEY

## UNITED STATES PATENT OFFICE

2,020,853

PHOTOGRAPHIC AMUSEMENT DEVICE AND  
METHOD OF MAKING THE SAME

Herbert Pels, New Rochelle, N. Y.

Application September 27, 1933, Serial No. 691,125

5 Claims. (Cl. 95—38)

My present invention relates generally to the photographic art, and has particular reference, coordinate, to a new and unique amusement device and to an improved method of making 5 invisible but restorable photographic impressions.

While I have herein illustrated and shall hereinafter describe the manner in which certain phases of my invention are applicable to the production of a new and entertaining amusement in 10 the nature of a guessing game or the like, it will be understood that, from many aspects, my invention has a far wider applicability.

Briefly, my invention relates to an improved method of creating a photographic print with a 15 bleached and totally invisible photographic impression thereon, the same being, however, readily restorable to visibility by subsequent treatment.

The invention is predicated upon the well-known ability of mercuric chloride to react with 20 silver to form what is believed to be a mixture of silver chloride and mercurous chloride. Silver particles suspended in a gelatinous emulsion are of dark coloration, while silver chloride and mercurous chloride are almost white. Accordingly, 25 this transformation affords a means for endeavoring to effect a "bleaching" of positive photographic impressions, the restoration of the impression being accomplished by the ability of sodium thiosulphate subsequently to reduce the 30 mercurous chloride to metallic mercury.

I have found, however, that the action of mercuric chloride upon the silver of an ordinary photographic print, while producing a certain amount of effacement of the impression, is quite 35 ineffective to produce a complete "bleaching" or obliteration of the impression, due probably to the fact that the silver chloride (or, in any event, the mixture of silver chloride and mercurous chloride) is not entirely white but has a slight 40 yellowish cast. Accordingly, a faint but distinct impression always seems to remain visible, due to the contrast between the white paper back and the not-quite-white mixture of particles of silver chloride and mercurous chloride. This contrast 45 is accentuated by the decided difference in textures between a layer or mass of these particles and the paper backing.

In accordance with my present invention, I am 50 enabled to "bleach" or render completely invisible a photographic impression, so that even the most painstaking scrutiny cannot discern the presence of any photographic impression whatsoever. In fact, a photographic print produced in accordance with my present invention has a surface 55 that is absolutely blank and devoid of even

the slightest trace of any impression; and the print may even be held between a source of light and the observer without revealing the fact that a predetermined photographic impression is carried thereby. This capability of the present invention leads to the possibility of providing a unique amusement device which consists essentially of a bleached but restorable photographic print, the print bearing an invisible photographic impression of a recognizable subject, and bearing 10 at the same time certain constantly visible indicia which afford clues to the identity of the subject. This photographic print is coupled with an extremely simple means for effecting a restoration of the visibility of the impression, whereby the 15 person employing the amusement device may preliminarily endeavor to guess the nature and identity of the subject subsequently capable of restoration to visibility by him. I contemplate that such amusement devices may be provided in 20 series, furnished, for example, as premiums with commercial products or the like, whereby children will not only seek to collect all the photographic prints of a given set or sets, but will be afforded the pleasure of indulging in an educational mystifying amusement in the restoration of each 25 print of the set.

One of the salient characteristics of my present invention resulting in the successful production of a totally complete invisibility of a 30 photographic impression, lies in the treatment, with mercuric chloride, of a silver-halide-emulsion layer which has been photographically impressed, developed, but not fixed. Chemically, as 35 is well-known, the development continues and completes the reduction of the silver-halide particles of the emulsion to metallic silver in varying degrees, depending upon the amount of light to which each particle has been subjected. Where such a layer is then immediately subjected to the action of mercuric chloride, the deposited silver is transformed back into silver chloride and forms a mixture with mercurous chloride. This mixture, I have found, is utterly indistinguishable, both in coloration and texture, from the 40 unreduced silver-halide portions of the emulsion. The resultant "invisibilized" print may thus be said to bear a photographic impression formed of a mixture of silver chloride and mercurous chloride, the balance of the print comprising a 45 layer of gelatine emulsion with suspended, unreduced, silver-halide particles therein.

The subsequent restoration of the visibility of the impression may then be expeditiously effected by merely treating the print with sodium thio- 55

sulphate, which serves simultaneously to deposit metallic mercury and to dissolve away all unreduced silver chloride and other silver-halide.

The characteristics of my invention will be 5 more fully appreciated upon reference to the accompanying drawing, in which—

Figure 1 is a view of an "invisibilized" print forming an element of the present amusement device;

10 Figure 2 is a view of a preferred means for restoring the print;

Figure 3 is a view similar to Figure 1, showing the print in final restored and permanent condition;

15 Figure 4 is an enlarged cross-sectional view through the print, illustrating diagrammatically the effect of exposure to the desired photographic impression and the subsequent development;

Figure 5 is a view similar to Figure 4, showing 20 diagrammatically the effect of the bleaching procedure; and

Figure 6 is a view similar to Figure 5, showing diagrammatically the effect of the restoration step.

25 While any desired or suitable backing may be employed, I have illustratively shown a paper backing 10 of conventional character, the paper being preferably of substantially smooth and uniform white character. On one surface it is provided with a layer 11 consisting of an emulsion of gelatine and silver-halides. Preferably, a chloro-bromide paper is employed, but any suitable so-called "developing-out" paper may be used.

30 In carrying out my present invention, the layer 11 is first subjected to the desired photographic impression which may, for example, be the portrait of a motion-picture actress, as indicated in Figure 3. The exposure of the paper is preferably, but not necessarily, accomplished by "contact printing", this being performed in a safe light. The print is then subjected to the usual development, for example, in an ordinary developer such as metol-hydroquinone. The exposure 35 and development result in the deposit of silver particles, for example, in the typical area 12 of Figure 4. When this procedure has progressed to the desired degree, the developing action is discontinued by preferably placing the print in a stop-bath composed, for example, of forty parts of water and one part of concentrated hydrochloric acid. The print is left in this bath for at least half a minute, and, if desired, for a longer period.

40 In the ordinary process of photographic printing, the print would thereupon be subjected to the action of "hypo" which would dissolve away all the unreduced silver salts of the emulsion, thereby "fixing" the impression on the backing 45 10.

50 In accordance with my invention, however, I scrupulously avoid any such procedure, and after rinsing the print briefly, I immerse it at once into a bath composed, preferably, of approximately four ounces of water, one-quarter ounce of concentrated hydrochloric acid, and sixty-five grains of mercuric chloride. The print is left in this bath until the image has completely disappeared, which ought to take about fifteen or twenty minutes. The disappearance of the image is absolute, and leaves not the slightest visible trace, being caused by the conversion of silver into a mixture of silver chloride and mercurous chloride. A mass of this mixture is 55 formed wherever there was previously a mass of

silver particles, as indicated by the area 12 of Figure 5. This area is utterly indistinguishable in texture and color from the balance of the emulsion which is composed of unreduced original silver salts.

60 After the print has been washed thoroughly to remove the mercuric chloride, the production of the completely "invisibilized" photographic print is accomplished, subject, of course, to a drying action which is caused to take place in the dark. The washing away of the mercuric chloride may be hastened, if desired, by successive baths of hydrochloric acid, one to forty, followed by washing in water; but in such a case, it is advisable to treat the print with a ten per cent solution 15 of formaldehyde for about twenty minutes, followed by a brief wash in water. The formaldehyde serves to compensate for the softening of the gelatine by the acid.

65 The bleached print, when dried, is then ready 20 to be dispensed and used as one element of the amusement device. Preferably, the print is enclosed in a red glassine or waxed paper envelope or the like to guard it against undue exposure to strong light.

70 In accordance with my invention, the print is caused to bear certain constantly visible indicia such as those indicated at 13 in Figure 1. These indicia may appear either on the obverse face of the print 14 or on the reverse face. They may 30 be of any desired character, preferably affording a number of clues as to the identity and character of the subject of the bleached and invisible photographic impression.

75 To effect a restoration of the visibility of the 35 impression, it is merely necessary to subject the print 14 to sodium thiosulphate, the chemical effect being indicated in Figure 6. The sodium thiosulphate reacts with the mercurous chloride to form metallic mercury, sodium chloride, and 40 probably sodium tetrathionate, the mercury being the only insoluble resultant ingredient. The mercury deposits itself in the form of particles along the same areas that had previously been occupied by mercurous chloride, one of these areas 45 being designated diagrammatically by the reference numeral 15 of Figure 6. It is this deposit of mercury particles which effects a restoration of the image. The sodium thiosulphate simultaneously dissolves away all silver salts, including the unreduced original silver-halides, whereby the layer 11, in those places where there is no deposit of mercury, consists of pure transparent gelatine. This permits the white of the 50 backing 10 to be visible, and produces the contrast of black and white that is typical of the ordinary photographic print. The print is thus simultaneously restored and fixed, and is in a permanent and lasting condition after the process has been completed, subject, of course, to a 55 suitable washing of the print and a drying thereof.

60 The application of the sodium thiosulphate, in carrying out the present amusement, is preferably accomplished by means of a sheet 16 of 65 absorbent material, such as inexpensive yellow manila paper which has been impregnated with a solution of approximately two ounces thiosulphate of soda and ten ounces of water. The paper is left in this solution for about five minutes and is then hung up to dry without rinsing.

65 The "invisibilized" print of Figure 1, with the indicia 13 associated therewith, and the impregnated sheet 16 of Figure 2 form the elements of 70 my present amusement device. When used, to 75

restore and render permanent the photographic print, it is merely necessary to soak the print 14 in clear water for about a minute; then to draw the sheet 16 rapidly through the water in order to wet it; and the sheet 16 is then brought into firm contact with the emulsion side of the print 14, preferably on a flat surface. A slight rubbing of the finger tips insures contact and removes air bubbles. The image appears almost immediately, but contact is preferably continued for about five minutes to insure permanence. The sheets are then separated, the sheet 16 being discarded, and the print 14 is then washed in several changes of water for about five minutes each and then permitted to dry. The result is indicated in Figure 3, and provides the user with a permanent card or print which may advantageously form one of a series that it is desirable to complete and own.

Wherever I have used the term "bleached" herein, or in the appended claims, it will be understood to refer to an image obliteration of the character herein described, and not to a mere lightening or discoloring action, as the term "bleaching" usually connotes. Similarly, my reference to the "immediate" subjection of the print to the mercuric chloride, following its development, is to be construed as signifying the absence of any intermediate procedure such as the conventional fixing of the impression.

In general, it will be understood that changes in the details, herein described and illustrated for the purpose of explaining the nature of my invention, may be made by those skilled in the art without departing from the spirit and scope of the invention as expressed in the appended claims. It is, therefore, intended that these details be interpreted as illustrative, and not in a limiting sense.

Having thus described my invention, and illustrated its use, what I claim as new and desire to secure by Letters Patent is—

1. The method of making a bleached but restorable photographic print, which consists in subjecting a layer of silver-halide emulsion to the desired photographic impression, developing the layer to complete the reduction of the affected silver-halide particles to the desired degree, and then immediately subjecting said layer to mercuric chloride to transform the deposited silver into a mixture of silver-halide and mercurous chloride, said mixture being indistinguishable from the unreduced silver-halide portions of said layer, whereby the impression is rendered invisible but restorable by subsequent reduction of the mercurous chloride.

2. The method of bleaching and restoring a photographic print, which consists in subjecting a layer of silver-halide emulsion to the desired photographic impression, developing the layer to complete the reduction of the affected silver-halide particles to the desired degree, then immediately subjecting said layer to mercuric chloride to transform the deposited silver into a mixture of silver-halide and mercurous chloride, said mixture being indistinguishable from the unreduced silver-halide portions of said layer, washing and drying the resultant bleached print, and subsequently subjecting the print to sodium thiosulphate to reduce the mercurous chloride to mercury and dissolve away all silver-halide, 15 whereby the print is simultaneously restored and fixed.

3. In the herein-described method of making a bleached but restorable photographic print, the step which consists in treating a developed but 20 unfixed silver-halide-emulsion layer with mercuric chloride so as to transform the deposited silver into a mixture of silver-halide and mercurous chloride, said mixture being indistinguishable from the unreduced silver-halide portions 25 of said layer.

4. The method of bleaching and restoring a photographic print, which consists in subjecting a layer of silver-halide emulsion to the desired photographic impression, developing the layer to 30 complete the reduction of the affected silver-halide particles to the desired degree, then immediately subjecting said layer to mercuric chloride to transform the deposited silver into a mixture of silver-halide and mercurous chlo- 35 ride, said mixture being indistinguishable from the unreduced silver-halide portions of said layer, washing and drying the resultant bleached print, impregnating and drying an absorbent sheet of material with sodium thiosulphate, and subsequently re-wetting and contacting the bleached print and the impregnated sheet, whereby the sodium thiosulphate reduces the mercurous chloride to mercury and simultaneously dissolves away all silver-halide, thereby restoring and fix- 45 ing the print.

5. As a new article of manufacture, a bleached but restorable photographic print, comprising a backing, a layer of silver-halide emulsion thereon, said layer bearing portions conforming to a pre-determined photographic impression, said portions comprising a mixture of silver chloride and mercurous chloride, the remainder of the layer comprising unreduced silver-halide.

HERBERT PELS.